

## UNITED STATES PATENT OFFICE

2,160,290

## WEAR RESISTING ALLOY

Robert W. Schlumpf, Houston, Tex., assignor to  
 Hughes Tool Company, Houston, Tex., a corporation of Delaware

No Drawing. Application January 31, 1938,  
 Serial No. 187,895

## 3 Claims. (Cl. 75—126)

This invention relates to wear resisting compounds of hard metals.

It is an object of the invention to provide an alloy which is adapted to withstand abrasion and wear.

I desire to provide a steel having alloyed therewith metals combined in such proportion as to make the resultant alloy capable of withstanding wear due to contact therewith of abrasive materials such as sand, shot and the like.

The alloy is particularly adapted for use in casting tubes employed as nozzles in sand blasting, and for the discharge therethrough of fluids containing abrasive materials.

I also desire to provide a composition of metals which, when molten, is fluid enough for ready casting into molds.

My composition consists of iron having therein carbon, tungsten, chromium, and boron in about the following proportions:

|          | Percent      |
|----------|--------------|
| Carbon   | 1.0 to 1.5   |
| Tungsten | 14.0 to 18.0 |
| Boron    | 0.5 to 2.0   |
| Chromium | 5.0 to 6.0   |

In the making of this alloy I find it economical to use high speed steel scrap. Such scrap is waste about a machine shop where tools made of steel having therein a certain percentage of tungsten carbide are used. Such tools become worn out and have to be discarded as waste. I find that if carbon, chromium and boron are added to make up an alloy approximately as set out above, a particularly wear resistant metal is produced.

The boron not only adds materially to the wear resisting qualities of the alloy, but is also valuable in making the same more fluid when molten. It is thus easily cast into the form of tubes or nozzles.

Heretofore, a hard quality of steel has been extensively employed for wear resisting purposes in nozzles of this character, but I find that when nozzles are made of my new alloy, such tools will last from three to four times as long as with the old composition.

My invention is particularly valuable in the making of nozzles to conduct the flow of mud through a well drill in deep well operations. The drilling mud has quantities of abrasive material therein and the mud discharging tubes in the drill head become worn frequently before the cutters upon the drill are worn out. This seriously impairs the operation of the drill, as the pressure of the drilling fluid is decreased and the operation of the drill thus affected.

The proportions of the metals may be varied within the limits noted without materially affecting the character of the resulting alloy.

## What I claim is:

1. A hard abrasion resisting alloy comprising a mixture of materials fused together in approximately the following proportions: chromium, 5.0% to 6.0%; boron, 0.5% to 2.0%; carbon, 1.0% to 1.5%; and tungsten, 14.0% to 18.0%; the balance iron, said alloy being capable of being cast only, and incapable of being forged or worked.

2. A wear resisting composition made up of iron having alloyed therewith chromium, approximately 5%; boron, 1.5%; carbon, 1% and tungsten, 16%, said composition being capable of being cast only.

3. An abrasion resisting discharge nozzle made of iron alloyed with about 1% to 1½% of carbon; 14% to 18% of tungsten; 0.5% to 2.0% of boron; and 5% to 6% of chromium, said nozzle being cast into form.

ROBERT W. SCHLUMPF.